

Feb. 22, 1944.

A. L. J. QUENEAU

2,342,368

ZINC METALLURGY

Filed May 17, 1941



Inventor:

AUGUSTIN LEON JEAN QUENEAU,  
by: *John E. Jackson* his Attorney.

## UNITED STATES PATENT OFFICE

2,342,368

## ZINC METALLURGY

Augustin Leon Jean Queneau, Peapack, N. J.

Application May 17, 1941, Serial No. 394,009

4 Claims. (Cl. 75—26)

In zinc metallurgy, it is not an entirely new conception to proceed by what may be termed a "flash reduction" operation for winning zinc from zinciferous metallurgical materials.

In accordance with such "flash reduction" procedure, oxidic zinc material, together with carboniferous reducing agent, is showered through an environment which is heated to temperatures above the reduction and volatilization temperatures of zinc, the reduction taking place in the freely falling charge while the particles are in suspension in the environment. The carbon must be present in sufficient excess to contact efficiently with the zinc oxide particles during their fall, so that reduction and volatilization of the zinc will proceed before the charge reaches the bottom of the reactant environment.

In carrying out the flash reduction process, it has been the practice to shower the zinc oxide-carbon mixture through a vertical columnar retort composed of a monolithic structure of essentially silicon carbide. The retort is fired externally, and preferably a reducing environment is maintained in the retort in order to facilitate the reduction of the zinc oxide while it is freely falling. Propane gas has been employed for the maintenance of this reducing atmosphere, a propane atmosphere apparently tending to reduce the amount of blue powder produced during the operation. The formation of this blue powder has been one detriment to the flash reduction operation as has been practiced heretofore. This has led to various proposals for conditioning and scrubbing the emergent zinc stream as it passes to the condenser to remove various suspensoids in the gas stream which appear to act as nuclei for blue powder production.

Additionally, it has been proposed to increase the reduction rate by using activated, or alpha, carbon as the reducing agent. In prior procedure, the efficiency of the process is found to be increased thereby.

These specialized provisions of the prior practice are required because of certain existent factors:

1. The presence of suspensoids in the exit gases is due to entrained soiled particles from the charge, the presence of partially condensed impurities originally present in the zinc oxide concentrates employed for the charge, and to unreacted carbon particles arising from the use of uncontrolled large excesses of carbon which are employed to assure the presence of a sufficient mass of carbon to effect the reduction.

2. The use of such uncontrolled large excesses

of carbon arises because of imperfect physical contact between the particles of zinc oxide and the particles of carbon.

3. This imperfect physical contact requires for efficiency a speeding up of the reduction speed, which is attained by the use of highly reactive (activated) carbon, materially increasing the cost of the procedure.

4. The life of the silicon carbide "flash" column is not sufficiently satisfactory to make a flash reduction procedure competitive with respect to costs, with standard vertical retort operations. In accordance with the present invention, the cause of the unsatisfactorily shortened life of the silicon carbide "flash columns" employed in "flash" reducing operations as practiced prior to the present invention, now is found to be due to the presence of materials associated with zinc oxide, which even though present in sufficiently small amounts so as to enable the zinc oxide being employed to be classed as "substantially pure" zinc oxide, nevertheless, under the conditions existing in the flash column where the entire charge is being made up of continuously swirling particles being continuously introduced into the "flash" column, which particles intimately engage the hot silicon carbide surfaces of the column and come into wiping contact therewith, such materials under these ideal conditions for reaction attack both the silicon carbide of the column and the binder employed to bond the silicon carbide during the manufacture of the column, the resulting reactions causing a markedly quick disintegration and deterioration of the column. Such materials are found to be, importantly, certain slag-forming materials normally present with zinc oxide produced from zinc ores or concentrates, among which materials may be mentioned, importantly, lime, magnesia, iron oxides, lead, cadmium, silver and alkalies, which under the conditions maintained in the retort, react with the silicon carbide to produce silicates of the respective metals.

While the silicon carbide shells which form the "flash" column in the usual type thereof are found to be destroyed with marked rapidity by the presence of even small amounts of such materials in the zinc oxide being reduced, the same type of attack is observed in the case of the silicon carbide bricks which have been employed in the construction of vertical retorts using briquetted charges of zinc oxide and carbon, although in such installations, the attack is much slower, as the conditions for reaction with silicon carbide are much less favorable than are the conditions ex-

istent in a flash reduction column. However, even in the carborundum brickwork of vertical zinc retorts, in time there becomes a very appreciable attack on the surfaces of the brick that are exposed to the briquetted charges being processed.

The procedure of the present improved process is found to obviate these, and other, difficulties which have made impracticable a process which should be an attractive procedure from the standpoint of costs, as well as the yield and purity of the condensed metal.

Certain features distinguish the present invention:

A. A careful purification of the zinc-bearing materials to eliminate associated impurities, thereby obviating the necessity for special conditioning or scrubbing of the zinc-bearing gases passing from the flash retort to the condenser.

B. The production and maintenance of a homogeneous and intimate contact of the reactive carbon with the oxidic component of the charge, to eliminate the necessity of utilizing specially prepared activated or alpha carbon.

C. An efficient utilization of retort residues for recovering any unreduced values therein.

D. The avoidance of expensive costly atmospheres in the flash column.

Further objects and advantages of the present invention will become apparent as the description proceeds and the features of novelty will be pointed out specifically in the appended claims; and while the invention will be described with specific reference to a flash reduction of zinciferous materials, particularly zinc oxide concentrates, it will be understood that it is of advantage in the operation of other zinc metallurgical processes, including the usual type of vertical retort practice.

The invention will be understood more readily by reference to the accompanying drawing, which illustrates a diagrammatic flow-sheet of the process.

The present process may be divided into several cooperating parts, the interrelationship of which will become apparent from a consideration of the accompanying drawing which illustrates a diagrammatic flow sheet of the entire process. These cooperating parts are indicated in the different stages set forth in the description which follows hereinafter.

#### *Preparation of the charge*

One of the important features of the present invention is the preparation of the charge for the reduction.

Zinc ores occur in nature mixed with gangue materials and usually carry too low a percentage of zinc to allow for economical treatment for reduction to metal or chemical compounds. The crude ores, therefore, are processed so as to yield high grade concentrates; in the case of sulphide ore, of 60 per cent zinc or better. Even these high grade zinc concentrates contain substantial amounts of contaminating chemical elements or compounds, such as sulphur, iron, silica, lime, cadmium, lead, etc.

In many instances, it is of economic interest to increase further the zinc contents of the mill concentrates mentioned above. Thus, the sulphur may be eliminated by suitable oxidizing treatment, such as roasting. In accordance with the present process, there are concentrated further the zinc contents of roasted zinc concentrates by the further elimination of the remaining impurities by a suitable pyro-metallurgical treatment described herein.

The roasted zinc concentrates containing as main impurities iron and/or manganese oxides, lead sulphate, and small amounts of cadmium and precious metals, in accordance with the present invention are mixed with a suitable proportion of carbonaceous material, such as coke or anthracite coal, or other carbonaceous material high in fixed carbon, and the resulting mixture is fed into an inclined rotary kiln of the general type used in the well-known Waelz process for producing zinc oxide. The heat gradient required for the operation is maintained principally by the combination of the fuel addition to the zinc ore charge and, in addition, if required, by a burner supplying additional heat through the burning of powdered coal, fuel oil, or other suitable fuel, the selection of the fuel supply for the burner being largely a question of convenience and costs.

In its passage through the rotary kiln, the zinc oxide is reduced within the body of the charge, tumbling and rolling in contact with the lower and rising part of the kiln lining, principally in accordance with the reaction:



As there is of necessity an excess of carbon present in the kiln charge, a secondary reaction also takes place:



The metallic zinc vapors, together with the carbon monoxide issuing from the highly heated charge, burn freely in contact with the current of highly heated air admitted at the discharge end of the kiln. It may be noted in passing that that heat liberated by the combustion of zinc vapor to zinc oxide and of the carbon monoxide to carbon dioxide is substantially equivalent to the amount of heat required for the reduction of zinc oxide in the roasted ore, with allowance for the heat which is carried away from the kiln by the gases of combustion, and also for the heat that must be supplied to the radiating outer surface of the kiln.

Now, as the vapors of the reduced zinc are burned, zinc oxide is re-formed. But now this zinc oxide is liberated almost completely freed from gangue impurities, except a small amount thereof that is carried as fine dust by the gas stream sweeping through the kiln to its exit. However, the resulting zinc oxide usually contains some lead, cadmium, and silver, since lead is reduced with the zinc and volatilizes as lead sulphide, which later oxidizes to lead sulphate. The cadmium follows the zinc, as well as a small percentage of the silver present in the original roasted ore or concentrate.

If the roasted ore or concentrate carries substantial values in gold and silver, the presence of copper in the kiln charge is of assistance in retaining the precious metals in a complex iron-copper matte which is an active absorber of gold and silver. If copper is absent in the zinc calcines, an addition of copper-bearing material to the charge may be found to be advantageous.

The initially purified zinc oxide is collected in any suitable way, as in textile bags, or in a Cottrell precipitator. This zinc oxide contains substantially all of the zinc content of the roasted ore charge with its lead and cadmium contents. It also includes a small amount of fine particles of gangue, of carbon, and also a comparatively large volume of sulphur dioxide and other gases occluded and adsorbed on the zinc oxide particles, so that further treatment of the zinc oxide is

required for the elimination of the lead, cadmium, silver, and the occluded gases.

For this purpose, the crude zinc oxide is mixed thoroughly with a halide compound, preferably sodium chloride. The resulting mixture is fed onto the bed of a blast sintering machine, such as a Dwight-Lloyd machine, with the salt present in the charge in slight excess of the stoichiometric requirements of the lead, cadmium, and silver. The charge is sintered.

This sintering removes all of the contaminating metals, lead, cadmium, and silver, as chlorides and/or sulphates, together with the whole of any sulphur present. These contaminants are carried away from the sinter bed by the gases sweeping at high velocity through the bed. The resulting gases pass through a suitable Cottrell precipitator in which the metal compounds are collected.

The sintering operation is carried on in such a way as to produce a light porous sintered product, this being obtained by adding to the charge of the sintering machine a strict minimum amount of fixed carbon, such as coke or anthracite coal, for minimizing the maximum temperature reached in the bed of the sintering machine.

The resulting sintered product consists of substantially pure zinc oxide which is highly suitable for further metallurgical treatment for the production of high grade zinc metal by flash or suspension reduction or in a vertical continuous retort, or other procedure.

The residual gangue matter in the rotary kiln charge is discharged at its lower end, together with any excess of carbon that may be present. If the kiln charge contained sufficient values of precious metals, together with an adequate amount of copper, the resulting complex iron-copper matte carrying the precious metals may be separated readily from the otherwise valueless slag by crushing and treatment by the usual ore-dressing methods, such as tabling, but preferably by flotation.

It will be seen, therefore, that from a complex zinc ore carrying gangue materials, such as iron, manganese, silica, lime, etc., together with additional metal values, such as lead, cadmium, and precious metals, there is effected a substantially complete separation of substantially pure zinc oxide, the final products consisting of:

1. A sintered, substantially pure zinc oxide.
2. A mixed cottrell dust or fume containing the original lead and cadmium contents of the ore.
3. A complex iron-copper matte containing the precious metal values of the zinc ore.

Now, this highly purified zinc oxide is to be mixed with a carbonaceous reducing agent, in accordance with standard procedures for flash reduction operations, with the exception that in accordance with the present improved process, there is produced a charge consisting essentially of a very intimate contact of the purified zinc oxide with controlled amounts of carbon.

In order to effect the improvements of the present process, the purified sintered zinc oxide prepared as above, together with coke, low-ash anthracite coal, or other carbonaceous material low in mineral matter, and in the proportion of about 100 parts by weight of the zinc oxide sinter to from about 20 to 25 parts by weight of the low-ash carbonaceous reducing material, are mixed together thoroughly while water-free hot tar is introduced into the mixture, the tar addi-

tions amounting to from about 15 parts by weight to about 20 parts by weight.

The mixture then is passed through a steam jacketed pug mill from which the thoroughly incorporated mixture is extruded in the form of a hollow cylinder six inches in diameter with one and one-half inch central perforation, and cut into twelve-inch lengths or briquettes. These briquettes are piled on a platform car and run into a tunnel furnace, heated indirectly, in which there is maintained a maximum temperature of from about 600° C. to 800° C., the briquettes being brought slowly to full temperature until all volatile matter has been expelled and the briquettes are coked.

The coked briquettes are crushed all through a one-inch screen, the crushed product then being fed to a rod mill operating in a closed circuit with an air classifier to give a final product, about 20 85 per cent of which passes through a 200-mesh screen.

The particles of this product consist principally of purified zinc oxide completely permeated with fixed carbon deposited during the distillation and coking of the briquettes. There is provided thereby completely intimate contact between the reducing material and the zinc oxide. This contact, it is to be emphasized, is not the haphazard contact between finite and separate particles of zinc oxide and carbon, as has been employed in reduction processes prior hereto, but, on the contrary, it is an actual finite zinc oxide-carbon contact existing within each concrete particle of zinc oxide, thus providing optimum conditions for the rapid reduction of the zinc oxide when these pulverized zinc oxide-coke briquettes are brought up to the required zones of temperature for reduction.

The charge of pulverized briquette material is passed into a preheater consisting of a rotary kiln which is fired externally and in which a temperature of from about 700° C. to about 800° C. is maintained.

#### Reduction of the charge

The charge, prepared as above, and heated to from about 700° C. to about 800° C. (the temperature may vary according to the nature and characteristics of the zinc oxide to be reduced), is continuously fed and showered into a vertical reducer furnace or retort composed of silicon carbide, maintained at a temperature of from about 1100° C. to about 1250° C., in which the reduction of the zinc oxide-carbon complex is effected principally according to the reaction:



Since, however, there is an excess of carbon at a glowing temperature in the furnace charge, the producer-gas reaction becomes effective:



The value of the presence of carbon particles in intimate contact with the zinc oxide of the sinter is indicated by Reaction 2.

It is known that the speed of Reaction 1 is faster than that of Reaction 2; consequently, it is of the utmost importance for the efficient reduction of zinc oxide in suspension, that all facilities be provided for supplying glowing carbon at the very point where  $\text{CO}_2$  is liberated.

The present process provides means for accomplishing this presence, since the carbon particles impregnating the zinc oxide sinter are present "in situ" at the point where the  $\text{CO}_2$  is liberated and when it should be reduced to CO as rapidly

as possible. The carbon present within each concrete particle of zinc sinter offers immediate contact with the liberated  $\text{CO}_2$ .

This is not the case when the carbon is present in the charge only as particles separate and distinct from the zinc calcine particles of the suspension zinc oxide furnace charge.

The zinc vapor, together with the carbon monoxide, with possibly a trace of carbon dioxide, may be passed through a conventional bed of glowing coke to bring a further reduction of such small percentage of residual  $\text{CO}_2$ , as well as the filtration of the suspended excess carbon and carbon ash. The purified gas and metallic zinc vapor stream pass to a usual type of plate condenser for zinc maintained at the optimum temperature for the condensation of the zinc vapor to liquid zinc.

The residual carbon monoxide stream, carrying a small proportion of zinc dust and blue powder, passes through a small column through which flows counter-currently a spray of water.

This collected zinc dust and blue powder mud (zinc dust, zinc oxide, and blue powder) is returned to the pug mill for a further treatment with the following charge of purified sintered zinc oxide, while the washed carbon monoxide issuing from the zinc condenser is utilized to provide a controlled non-oxidizing atmosphere in both the coking briquette furnace and the pre-heating rotary kiln for the charge of pulverized briquettes of zinc oxide-carbon. The carbon monoxide, after its passage through both furnaces, is burned to supply additional heat units in both furnaces.

In the flash reduction furnace, there may be provided an incandescent column of coke, although the presence thereof is not obligatory by any means. But where such coke column is provided, its temperature is at the high heat level required (1200° C.-1300° C.), which is maintained by indirect heating, as when adjacent to the flash reduction furnace wall, by electrical resistance, or by direct partial combustion by the admittance at a point above the bottom of the coke column of a strictly metered amount of atmospheric air.

The sized coke (all through a 2-inch ring and plus  $\frac{3}{4}$  inch) is fed to the coke column at a continuous rate through a gas-tight seal and there is withdrawn at an equal rate and continuously an equal amount from the foot of the column also through a gas-tight seal, and quenched. The coke also may be supplied to the reduction furnace in the form of briquettes.

As has been pointed out above, the present invention provides means for maintaining carbon in intimate contact with the zinc oxide of the charge; and it has been pointed out above that the reduction of the zinc oxide proceeds in accordance with the two reactions:



The gaseous products of the reduction reactions of the suspension zinc furnace, CO, zinc vapor, and possibly traces of  $\text{CO}_2$ , together with any unreduced zinc oxide of the charge, the gangue material of the sintered ore charge, and excess coke of the charge, are brought into intimate contact with the incandescent coke column. The gases and metallic vapors filter through the coke column; any  $\text{CO}_2$  present is reduced by the incandescent carbon to CO in accordance with the gas producer reaction:



This reaction is an exothermic reaction and all the solids are entrapped by and within the coke column.

These residual solids finally are withdrawn from the reduction furnace, together with the coke that is being withdrawn continuously. The withdrawn solids, coke, and residues, are screened, all material passing a  $\frac{3}{4}$ -inch screen is separated, and the  $+\frac{3}{4}$ -inch coke is returned to the feed of the coke column, while all  $-\frac{1}{2}$ -inch material is crushed and passed to the feed of the rotary kiln as reducing and heating fuel. The  $-\frac{3}{4}$ -inch and  $+\frac{1}{2}$ -inch material is sent to a crusher for addition as fuel to the reduction furnace charge preparatory to the tar addition.

The coke fines also carry the residues from the zinc charge of the suspension zinc reduction furnace. These fines pass to the rotary kiln and are mixed with the incoming charge of crude zinc ore calcines and coke.

This procedure enables the residual zinc values to be utilized, together with the withdrawn undersized coke.

These purified zinc vapors and gases now consisting substantially wholly of carbon monoxide with a small percentage of nitrogen (from the air, admitted in regulated amount to the base of the incandescent coke column), pass to the condenser wherein the zinc vapor is condensed to liquid metal. The residual gases, mainly CO, issuing from the scrubbing tower of the zinc condenser, are returned in the volume required to the top of the flash reduction furnace to provide the carbon monoxide atmosphere required for the zinc reduction process and are preheated to 1000° C.-1100° C. before admission to the furnace. The admission of a regulated amount of air at the base of the incandescent coke column serves the further purpose in helping to scavenge and evacuate therefrom any zinc vapor that might have a tendency to concentrate at the bottom of the furnace within the coke column. This function is in addition to its assisting in maintaining the temperature of the coke column at the level desired.

After passage through the zinc condenser, the residual gases and zinc vapors go through an adjacent scrubbing tower in which flows counter-currently a spray of water to collect all remaining solid particles that have escaped collection and settling in the condenser. Any uncondensed zinc vapor is oxidized partly or wholly in the scrubbing tower and is collected as a mud consisting of zinc oxide and zinc dust. The product is removed at intervals from the bottom settling tank, which also forms a gas seal.

The clean residual gases, which consist principally of carbon monoxide, pass through a pre-heater, a portion thereof passing thence to the preheating furnace in which the finely comminuted charge of the suspension zinc reduction furnace is brought to a temperature of 800° C.-900° C. before introduction to the flash reduction furnace.

The following products are obtained from the flash reduction:

1. Zinc ingots or slabs.
2. Zinc dust as metallic mud from the base of the condenser scrubbing column at its exit.
3. Zinc-bearing coke withdrawn from the coke column and zinc-bearing residues from the reduction furnace.

The metallic zinc dust and mud from the condenser scrubbing tower pass to the conditioning

pug mill in which the zinc oxide sinter is mixed with coke and hot anhydrous tar, as has been described above, for further treatment in the flash furnace.

Product 3, above, passes to the rotary kiln for the recovery of the zinc and carbon contained therein. The product is mixed with fresh incoming ore, and the resulting zinc oxide passes to the sintering stage for refining, thence to the pug mill and back to the flash furnace, as has been described above.

Where the coke column is omitted from the furnace, the residual discharge is correspondingly different, the furnace residues being passed to the rotary kiln, as described above, in the presence of carbon admixed therewith. Also, additional precautions must be taken to assure the producer gas reaction proceeding in the flash column through interaction of the carbon of the charge with any carbon dioxide tending to be formed, which, however, cannot exist as such. Consequently, sufficient carbon in the charge must be provided to maintain the gas producer Reaction 2, above, for minimizing blue powder formation. Also, of course, the elimination of the coke column obviates introduction of air into the environment in the flash reduction shaft. Otherwise, the operation is in accordance with the description given above.

The following illustrative data show the results obtained in the preparation of the zinc oxide for charging.

A zinc sulphide concentrate assaying Zn 61.77 per cent; S 30.82 per cent; Fe 1.15 per cent; Pb 1.12 per cent; Cd 0.389 per cent; CaO 0.10 per cent; MgO 0.594 per cent; SiO<sub>2</sub> 3.26 per cent; Al<sub>2</sub>O<sub>3</sub> 0.51 per cent, first was roasted.

The roasted concentrate analyzed: Zn 71.30 per cent; S 2.55 per cent; Pb 0.31 per cent; Cd 0.03 per cent; Fe 1.69 per cent; CaO 0.29 per cent; MgO 0.70 per cent; SiO<sub>2</sub> 5.34 per cent; Al<sub>2</sub>O<sub>3</sub> 0.60 per cent; O 17.45 per cent.

This roasted concentrate was charged into the rotary kiln and the zinc oxide produced by the kiln in a procedure similar to the well known Waelz process.

This zinc oxide analyzed; ZnO 87.0 per cent (Zn 69.8 per cent); S 2.0 per cent; Pb 0.03 percent; Cd 0.31 per cent; SiO<sub>2</sub>.Al<sub>2</sub>O<sub>3</sub> 4.00 per cent; CaO.MgO 0.50 per cent; C 6.14 per cent.

This oxidic material then is sintered in the presence of salt, as described above, prior to the mixing with tar in the pug mill. The sintered product analyzed: ZnO 94.80 per cent; SiO<sub>2</sub>.Al<sub>2</sub>O<sub>3</sub> 4.60 per cent; CaO.MgO 0.60 per cent.

The zinc recovered in the condenser on the flash reduction unit averages about 95 per cent of the zinc content of the original material.

A reducing atmosphere must be maintained in the reduction environment, the atmosphere being preferably carbon monoxide, since the use of other reducing gases (e. g., hydrocarbons, such as propane) may tend to produce water in the system by interaction with the carbon dioxide resulting from the reduction of the zinc, thus enhancing the formation of blue powder. Since carbon monoxide is the principal reducing agent for the zinc, the use of the carbon monoxide atmosphere introduces no extraneous material into the reacting system; and with the intimate contact between the carbon and the zinc oxide, which is provided by the present invention, there are provided optimum conditions for the maintenance of the producer gas reactions.

While the coke column may be omitted, its use as described herein, is preferred.

I claim:

1. The process of producing zinc, which comprises converting an impure zinciferous material into substantially pure zinc oxide free from cadmium, lead, silver, and all other materials chemically reactive towards silicon carbide, preparing a charge of the said pure zinc oxide by intimately mixing it with a substantially anhydrous bituminous material including water-free tar, kneading the tar until complete impregnation with the tar is effected, heating the resulting mixture to a coking temperature until the bituminous material is coked in situ in the zinc oxide, finely comminuting the resulting material, maintaining the coke and oxide in continuous contact, showering the resulting mixture through a flash reduction environment having surfaces in contact with the material composed of silicon carbide heated to reducing temperatures, and effecting a reduction of the charge to elemental zinc while the charge is in free movement in the environment.

2. The process of producing zinc which comprises converting an impure zinciferous material into a substantially pure zinc oxide free from materials chemically reactive towards silicon carbide, preparing a charge of the said pure zinc oxide by intimately mixing it with a bituminous material adapted to form coke upon heating to coking temperature, kneading together the bituminous material and the pure zinc oxide until complete intermixing results, heating the resulting mixture to coking temperature until the bituminous material is coked in situ in the zinc oxide, finely comminuting the resulting material maintaining the coke and oxide in continuous contact, showering the resulting mixture through a flash reduction environment having surfaces in contact with the mixture composed of silicon carbide heated to reducing temperatures, and effecting a reduction of the charge to elemental zinc while the charge is in free movement in the environment.

3. The process of producing zinc which comprises converting an impure zinciferous material into a substantially pure zinc oxide free from materials chemically reactive towards silicon carbide, preparing a charge of the said pure zinc oxide by intimately mixing it with a bituminous material adapted to form coke upon heating to coking temperature, kneading together the bituminous material and the pure zinc oxide until complete intermixing results, heating the resulting mixture to coking temperature until the bituminous material is coked in situ in the zinc oxide, finely comminuting the resulting material maintaining the coke and oxide in continuous contact, showering the resulting mixture through a flash reduction environment having surfaces in contact with the mixture composed of silicon carbide heated to reducing temperatures, and effecting a reduction of the charge to elemental zinc while the charge is in free movement in the environment.

4. The process of producing zinc which comprises converting an impure zinciferous material into a substantially pure zinc oxide free from materials chemically reactive towards silicon carbide, preparing a charge of the said pure zinc oxide by intimately mixing it with a bituminous material adapted to form coke upon heating to coking temperature, kneading together the bituminous material and the pure zinc oxide until complete intermixing results, heating the resulting mixture to coking temperature until the bituminous material is coked in situ in the zinc oxide, finely comminuting the resulting material maintaining the coke and oxide in continuous contact, showering the resulting mixture through a flash reduction environment having surfaces in contact with the mixture composed of silicon carbide heated to reducing temperatures, and effecting a reduction of the charge to elemental zinc while the charge is in free movement in the environment.

5. The process of producing zinc which comprises converting an impure zinciferous material into a substantially pure zinc oxide free from materials chemically reactive towards silicon carbide, preparing a charge of the said pure zinc oxide by intimately mixing it with a bituminous material adapted to form coke upon heating to coking temperature, kneading together the bituminous material and the pure zinc oxide until complete intermixing results, heating the resulting mixture to coking temperature until the bituminous material is coked in situ in the zinc oxide, finely comminuting the resulting material maintaining the coke and oxide in continuous contact, showering the resulting mixture through a flash reduction environment having surfaces in contact with the mixture composed of silicon carbide heated to reducing temperatures, and effecting a reduction of the charge to elemental zinc while the charge is in free movement in the environment.

6. The process of producing zinc which comprises converting an impure zinciferous material into a substantially pure zinc oxide free from materials chemically reactive towards silicon carbide, preparing a charge of the said pure zinc oxide by intimately mixing it with a bituminous material adapted to form coke upon heating to coking temperature, kneading together the bituminous material and the pure zinc oxide until complete intermixing results, heating the resulting mixture to coking temperature until the bituminous material is coked in situ in the zinc oxide, finely comminuting the resulting material maintaining the coke and oxide in continuous contact, showering the resulting mixture through a flash reduction environment having surfaces in contact with the mixture composed of silicon carbide heated to reducing temperatures, and effecting a reduction of the charge to elemental zinc while the charge is in free movement in the environment.

7. The process of producing zinc which comprises converting an impure zinciferous material into a substantially pure zinc oxide free from materials chemically reactive towards silicon carbide, preparing a charge of the said pure zinc oxide by intimately mixing it with a bituminous material adapted to form coke upon heating to coking temperature, kneading together the bituminous material and the pure zinc oxide until complete intermixing results, heating the resulting mixture to coking temperature until the bituminous material is coked in situ in the zinc oxide, finely comminuting the resulting material maintaining the coke and oxide in continuous contact, showering the resulting mixture through a flash reduction environment having surfaces in contact with the mixture composed of silicon carbide heated to reducing temperatures, and effecting a reduction of the charge to elemental zinc while the charge is in free movement in the environment.

8. The process of producing zinc which comprises converting an impure zinciferous material into a substantially pure zinc oxide free from materials chemically reactive towards silicon carbide, preparing a charge of the said pure zinc oxide by intimately mixing it with a bituminous material adapted to form coke upon heating to coking temperature, kneading together the bituminous material and the pure zinc oxide until complete intermixing results, heating the resulting mixture to coking temperature until the bituminous material is coked in situ in the zinc oxide, finely comminuting the resulting material maintaining the coke and oxide in continuous contact, showering the resulting mixture through a flash reduction environment having surfaces in contact with the mixture composed of silicon carbide heated to reducing temperatures, and effecting a reduction of the charge to elemental zinc while the charge is in free movement in the environment.

9. The process of producing zinc which comprises converting an impure zinciferous material into a substantially pure zinc oxide free from materials chemically reactive towards silicon carbide, preparing a charge of the said pure zinc oxide by intimately mixing it with a bituminous material adapted to form coke upon heating to coking temperature, kneading together the bituminous material and the pure zinc oxide until complete intermixing results, heating the resulting mixture to coking temperature until the bituminous material is coked in situ in the zinc oxide, finely comminuting the resulting material maintaining the coke and oxide in continuous contact, showering the resulting mixture through a flash reduction environment having surfaces in contact with the mixture composed of silicon carbide heated to reducing temperatures, and effecting a reduction of the charge to elemental zinc while the charge is in free movement in the environment.

10. The process of producing zinc which comprises converting an impure zinciferous material into a substantially pure zinc oxide free from materials chemically reactive towards silicon carbide, preparing a charge of the said pure zinc oxide by intimately mixing it with a bituminous material adapted to form coke upon heating to coking temperature, kneading together the bituminous material and the pure zinc oxide until complete intermixing results, heating the resulting mixture to coking temperature until the bituminous material is coked in situ in the zinc oxide, finely comminuting the resulting material maintaining the coke and oxide in continuous contact, showering the resulting mixture through a flash reduction environment having surfaces in contact with the mixture composed of silicon carbide heated to reducing temperatures, and effecting a reduction of the charge to elemental zinc while the charge is in free movement in the environment.

11. The process of producing zinc which comprises converting an impure zinciferous material into a substantially pure zinc oxide free from materials chemically reactive towards silicon carbide, preparing a charge of the said pure zinc oxide by intimately mixing it with a bituminous material adapted to form coke upon heating to coking temperature, kneading together the bituminous material and the pure zinc oxide until complete intermixing results, heating the resulting mixture to coking temperature until the bituminous material is coked in situ in the zinc oxide, finely comminuting the resulting material maintaining the coke and oxide in continuous contact, showering the resulting mixture through a flash reduction environment having surfaces in contact with the mixture composed of silicon carbide heated to reducing temperatures, and effecting a reduction of the charge to elemental zinc while the charge is in free movement in the environment.

12. The process of producing zinc which comprises converting an impure zinciferous material into a substantially pure zinc oxide free from materials chemically reactive towards silicon carbide, preparing a charge of the said pure zinc oxide by intimately mixing it with a bituminous material adapted to form coke upon heating to coking temperature, kneading together the bituminous material and the pure zinc oxide until complete intermixing results, heating the resulting mixture to coking temperature until the bituminous material is coked in situ in the zinc oxide, finely comminuting the resulting material maintaining the coke and oxide in continuous contact, showering the resulting mixture through a flash reduction environment having surfaces in contact with the mixture composed of silicon carbide heated to reducing temperatures, and effecting a reduction of the charge to elemental zinc while the charge is in free movement in the environment.

13. The process of producing zinc which comprises converting an impure zinciferous material into a substantially pure zinc oxide free from materials chemically reactive towards silicon carbide, preparing a charge of the said pure zinc oxide by intimately mixing it with a bituminous material adapted to form coke upon heating to coking temperature, kneading together the bituminous material and the pure zinc oxide until complete intermixing results, heating the resulting mixture to coking temperature until the bituminous material is coked in situ in the zinc oxide, finely comminuting the resulting material maintaining the coke and oxide in continuous contact, showering the resulting mixture through a flash reduction environment having surfaces in contact with the mixture composed of silicon carbide heated to reducing temperatures, and effecting a reduction of the charge to elemental zinc while the charge is in free movement in the environment.

14. The process of producing zinc which comprises converting an impure zinciferous material into a substantially pure zinc oxide free from materials chemically reactive towards silicon carbide, preparing a charge of the said pure zinc oxide by intimately mixing it with a bituminous material adapted to form coke upon heating to coking temperature, kneading together the bituminous material and the pure zinc oxide until complete intermixing results, heating the resulting mixture to coking temperature until the bituminous material is coked in situ in the zinc oxide, finely comminuting the resulting material maintaining the coke and oxide in continuous contact, showering the resulting mixture through a flash reduction environment having surfaces in contact with the mixture composed of silicon carbide heated to reducing temperatures, and effecting a reduction of the charge to elemental zinc while the charge is in free movement in the environment.

into the zinc oxide until thorough impregnation of the zinc oxide with the tar is effected, heating the resulting mixture to a coking temperature until the bituminous material is coked in situ in the zinc oxide, finely comminuting the resulting material, maintaining the coke and oxide in continuous contact, showering the resulting

5 mixture through a flash reduction environment having surfaces in contact with the material composed of silicon carbide heated to reducing temperatures, and effecting a reduction of the charge to elemental zinc while the charge is in free movement in the environment.

AUGUSTIN LEON JEAN QUENEAU.